# EUROPEAN PATENT SPECIFICATION

(11) **EP 3 890 856 B1**
(45) Date of publication and mention of the grant of the patent: **10.04.2024**
(21) Application number: 18830730.0
(22) Date of filing: 03.12.2018
(51) Int. Cl.: A63H 33/00

(54) **METHOD FOR CASTING A GEL OBJECT**
VERFAHREN ZUM GIESSEN EINES GELOBJEKTS
PROCÉDÉ POUR COULER UN OBJET EN GEL

(43) Date of publication of application: 13.10.2021
(73) Proprietor: Five Stars H.K. Ltd., Lai Chi Kok, Kowloon, Hong Kong (HK)
(72) Inventor: POON, Shiu, Chung, 7651 DH Tubbergen (NL); SJOERS, Martinus Cornelis, 7651 DH Tubbergen (NL)
(74) Representative: Patent Business B.V.
(86) International application number: PCT/EP2018/083391
(87) International publication number: WO 2020/114574

(56) References cited:
- EP-A2- 0 183 344
- US-A- 3 975 480
- US-A- 4 299 790
- US-A- 4 466 937
- US-A1- 2008 241 312
- US-B1- 6 485 771

## Description

### Field of the invention

The invention relates to a method for casting a gel object, a casting gel composition, kit of parts thereof, and a casting mould for casting a gel object.

### Background of the invention

For times, many materials like plaster, plastic and other materials have been casted into moulds. Often, these castings and casting methods were provided in a hobby and children's play setting.

Alternative materials and casting mould applications have been developed. For instance, the patent US4 299 790 A discloses in its title "a method and composition for forming a plaster object". According to the abstract, the patent relates to "Formation of toy figurines from tap water and a moldable mixture of calcium sulphate hemihydrate with xanthan gum in a shaker molding assembly. The molded article dries into a porous lightweight object. The materials are non-toxic."

### Summary of the invention

Hence, it is an aspect of the invention to provide an alternative casting method, kit-of-parts and casting mould. In particular, there is provided a children's paly assembly of kit-of-parts, which preferably further at least partly obviates one or more of above-described drawbacks.

There is currently provided a method according to claim 1.

There is further provided a kit-of-parts according to claim 5.

It was found that the method provides a new and attractive playing experience to children, for instance. The design of the casting mould in combination with specific casting gels allows creation of for instance multi-coloured objects. The compositions can be provided in such a way that they gel or form a gel fast, providing a food-grade or almost gel object. This provides a good play and educational experience for children. The special mould allows creative combining of colours, and teaches thinking in process steps.

In an embodiment, a water-soluble alginate is used. In particular, sodium alginate is used as one of the gelling compounds. Other, preferably child-save and for instance food-save alginates can be used, and that are known to a skilled person to have comparable properties. Sodium alginate, however, is relatively cheap, and safe to use.

In general, sodium alginate is a salt from alginic acid, also called algin or alginate. Alginic acid is a linear copolymer with homopolymeric blocks of (1-4)-linked β-D-mannuronate (M) and its C-5 epimer α-L-guluronate (G) residues, respectively, covalently linked together in different sequences or blocks. The monomers can appear in homopolymeric blocks of consecutive G-residues (G-blocks), consecutive M-residues (M-blocks) or alternating M and G-residues (MG-blocks).

Alginates are often refined from brown seaweeds. A wide variety of brown seaweeds of the class Phaeophyceae are harvested throughout the world to be converted into the raw material commonly known as sodium alginate

In an embodiment of the current invention, this is provided in an aqueous composition, in particular in combination with a colorant like a dye, a pigment, or a combination thereof.

Example, non-limiting, of possible colorants are: Pigment blue 15 (CAS no. 147-14-8), Pigment Green 7 (CAS no. 1328-53-6), Pigment Yellow 14 (CAS no. 5468-75-7), Pigment Yellow 23 (CAS no. 1934-21-0), Pigment Violet 23 (CAS no. 6358-30-1), Pigment Red 48 (CAS no. 3564-21-4), Pigment Red 170 (CAS no. 5858-81-1), Pigment Orange 13 (CAS no. 3520-72-7). These colorants are usually added in weight percentages of between 0.2-1.0. In an embodiment, these are used in amounts of between 0.25-0.85 on weight.

The colorant can also be or comprise a pigment, like for instance titanium dioxide (CAS no. 13463-67-7). Titanium dioxide and similar pigments are usually applied in percentage on weight of between 0.1-0.01. In an embodiment, these are used in quantities of between 0.05 and 0.015 on weight. Other, similar pigments can be used, either in natural form of treated in order to be compatible with the further composition in which they are used.

Furthermore, additional additives may be added for compatibility, or as preservatives, like for instance sodium benzoate, methylparaben, or similar substances that are known to a skilled person. These are used in quantities known to a skilled person, and in compliance with legislation of children's toys, and possibly food regulations.

In an embodiment, the gel-forming composition is provided as basically two compounds which, when brought into contact producing a gel, in particular an aqua gel. One of these two compounds is provided in various compositions, each having a different colour, and one can be colourless. These compounds are provided as a kit of parts.

In an embodiment of the method, the at least two gel-forming compositions have different colours, in particular including colourless one colourless gel-forming composition.

In an embodiment of the method, providing said at least two gel-forming compositions comprises providing:
- at least two first aqueous compositions comprising a water-solvable salt of an alginic acid and at least one of a respective first and second colouring agent or colorant;
- a second aqueous composition comprising at least 0.5-10 % by wt. calcium chloride, and
- contacting said at least two first aqueous compositions and said second aqueous composition.

In an embodiment the method further comprises:
- filling said at least one second casting mould sub volume with a first of said first aqueous solution;
- filling said first casting mould sub volume with a second of said first aqueous solution, and
- contacting said first aqueous solutions in said casting mould with said second aqueous solution.

In an embodiment, the casting mould comprises a series of second casting mould sub volumes that are each separated from said first casting mould sub volume via a said separating wall.

In an embodiment, the casting mould sub volumes each comprise a casting mould sub volume floor, wherein in particular said a casting mould sub volume floors is raised a maximum of 20 % of the outer wall height with respect to a neighbouring sub volume floor.

In an embodiment, at least one sub volume comprises an indent or hole, in particular having a depth of between 1-0.25 times the separating wall height.

In an embodiment, the casting mould has a ratio of casting mould diameter to casting mould outer wall height of between 1:1 to 20:1, and a ratio of casting mould outer wall height to separating wall height of between 3:1 to 3:2.

In an embodiment, the casting mould diameter is between 3 and 15 cm, in particular between 5 and 9 cm.

In an embodiment, the at least two first aqueous compositions each comprises at least one colouring agent providing said two first aqueous compositions with a visually different colour.

In an embodiment, the at least two first aqueous compositions are partially gelled, in particular said at least two first aqueous compositions are each provided in a tube and gelled such that they need to be pressed out of their tube by mild pressure, for instance by hand.

The term "substantially" herein, such as in "substantially consists", will be understood by the person skilled in the art. The term "substantially" may also include embodiments with "entirely", "completely", "all", etc. Hence, in embodiments the adjective substantially may also be removed. Where applicable, the term "substantially" may also relate to 90% or higher, such as 95% or higher, especially 99% or higher, even more especially 99.5% or higher, including 100%. The term "comprise" includes also embodiments wherein the term "comprises" means "consists of'.

The term "functionally" will be understood by, and be clear to, a person skilled in the art. The term "substantially" as well as "functionally" may also include embodiments with "entirely", "completely", "all", etc. Hence, in embodiments the adjective functionally may also be removed. When used, for instance in "functionally parallel", a skilled person will understand that the adjective "functionally" includes the term substantially as explained above. Functionally in particular is to be understood to include a configuration of features that allows these features to function as if the adjective "functionally" was not present. The term "functionally" is intended to cover variations in the feature to which it refers, and which variations are such that in the functional use of the feature, possibly in combination with other features it relates to in the invention, that combination of features is able to operate or function. For instance, if an antenna is functionally coupled or functionally connected to a communication device, received electromagnetic signals that are receives by the antenna can be used by the communication device. The word "functionally" as for instance used in "functionally parallel" is used to cover exactly parallel, but also the embodiments that are covered by the word "substantially" explained above. For instance, "functionally parallel" relates to embodiments that in operation function as if the parts are for instance parallel. This covers embodiments for which it is clear to a skilled person that it operates within its intended field of use as if it were parallel.

Furthermore, the terms first, second, third and the like in the description and in the claims, are used for distinguishing between similar elements and not necessarily for describing a sequential or chronological order. It is to be understood that the terms so used are interchangeable under appropriate circumstances and that the embodiments of the invention described herein are capable of operation in other sequences than described or illustrated herein.

It should be noted that the above-mentioned embodiments illustrate rather than limit the invention, and that those skilled in the art will be able to design many alternative embodiments without departing from the scope of the appended claims. In the claims, any reference signs placed between parentheses shall not be construed as limiting the claim. Use of the verb "to comprise" and its conjugations does not exclude the presence of elements or steps other than those stated in a claim. The article "a" or "an" preceding an element does not exclude the presence of a plurality of such elements. The mere fact that certain measures are recited in mutually different dependent claims does not indicate that a combination of these measures cannot be used to advantage.

The invention further applies to an apparatus or device comprising one or more of the characterising features described in the description and/or shown in the attached drawings. The invention further pertains to a method or process comprising one or more of the characterising features described in the description and/or shown in the attached drawings.

The various aspects discussed in this patent can be combined in order to provide additional advantages. Furthermore, some of the features can form the basis for one or more divisional applications.

### Brief description of the drawings

Embodiments of the invention will now be described, by way of example only, with reference to the accompanying schematic drawings in which corresponding reference symbols indicate corresponding parts, and in which:
Figure 1 schematically depicts an embodiment of a casting mould, and
Figure 2 schematically depicts an example of a cast gel object having various coloured parts, i.e., a main body and sub bodies.

The drawings are not necessarily on scale.

### Description of preferred embodiments

Figure 1 schematically depicts a casting mould 1. The casting mould 1 is surrounded by an outer casting mould wall 4 around the complete casting mould 1, defining a casting mould volume.

The casting mould 1 has a volume defined by the outer wall 4 that is divided into a first (here main) casting mould sub volume 2. The casting mould 1 further comprises in this example various second casting mould sub volumes 3. The first casting mould sub volume 2 has a first casting mould sub volume floor 5. The second casting mould sub volumes 3 each have a second casting mould sub volume floor 7. In most embodiments, the casting mould floor 5 and the casting mould sub volumes floors are substantially at a same level. Differences in level of neighbouring sub volumes floors are less than 10% of an outer wall height H. The casting mould outer wall 4 extends to a casting mould outer wall height H above the first casting mould sub volume floor.

The first sub volume 2 and the second sub volumes 3 are separated from one another by a separating wall having a separating wall height S.

In an example, for play objects like the current drawings, the casting mould 1 can be between 2 and 15 cm at its largest diameter. Often, the mould is about 5-10 cm at its largest diameter. In such embodiments, the casting mould outer wall 4 has a first outer casting mould wall height of between 2 and 10 mm (with respect to its floor). In the embodiment of 5-10 cm, the height will be about 3-6 mm.

The separating wall 6 has a separating wall height S of between about 1-4 mm. Usually it is between 35%-65% of the casting mould outer wall height.

In the illustrated example which has a largest diameter of about 5-10 cm, the first separating wall height S is between 45% and 55 % of the indicated height range of 3-6 mm.

The indicated indents 8 usually have a indent depth D with respect to the respective casting mould sub volume floor that is comparable to the separating wall height. The indent depth D for the illustrated example dimensions will be between 1 and 3 mm.

It is clear that in the casting mould sub volume, it is also possible to provide additional indents 8.

In use, in the method for making a gel object 10 (see figure 2 for the end product), first the indents 8 and casting mould sub volumes 3 are filled with an amount of gel-forming composition in different or identical colours (or even colourless..). Next, the first casting mould volume 2 is filled with a different colour of gel-forming composition. In an embodiment, the casting mould is first filled with different sodium alginate-comprising compositions, and the filled casting mould is subsequently contacted with a gel-inducing composition, for instance a calcium chloride comprising aqueous solution. After several seconds already, the gel object can be removed from the casting mould. The result is a multi-coloured gel object 10. The gel object 10 has a main body 11 formed in the first casting mould sub volume 2. The gel object 10 further has sub bodies 12 that are attached to the main body 11 and that are formed in the second casting mould sub volumes 3. The gel object con further have parches 13 that are formed in the indents 8. Thus, a colourful gel object can for instance be made. Despite the separating walls 6, the gel object is one single object.

### Example of a gel composition and kit-of-parts

### Component 1

| INCI name | CAS No. | Amount (% by Weight)* |
|---|---|---|
| Water | 7732-18-5 | 97.99-95.5 |
| SODIUM ALGINATE | 9005-38-3 | 2.0 |
| SODIUM BENZOATE | 532-32-1 | 0.3 |
| METHYLPARABEN | 99-76-3 | 0.2 |
| PHENOXYETHANOL | 122-99-6 | 0.5 |
| Colorant/pigment/dye | | 0.01-1.5 |

| | | |
|---|---|---|
| (*)The total amount adding up to 100% | | |

The colorant can for instance comprise:
Pigment blue 15 (CAS no. 147-14-8), Pigment Green 7 (CAS no. 1328-53-6), Pigment Yellow 14 (CAS no. 5468-75-7), Pigment Yellow 23 (CAS no. 1934-21-0), Pigment Violet 23 (CAS no. 6358-30-1), Pigment Red 48 (CAS no. 3564-21-4), Pigment Red 170 (CAS no. 5858-81-1), Pigment Orange 13 (CAS no. 3520-72-7). These colorants are usually added in weight percentages of between 0.2-1.0. In an embodiment, these are used in amounts of between 0.25-0.85 om weight.

TITANIUM DIOXIDE (CAS no. 13463-67-7). Titanium dioxide and similar pigments are usually applied in percentage on weight of between 0.1-0.01. In an embodiment, these are used in quantities of between 0.05 and 0.015 on weight.

### Component 2

| INCI name | CAS No. | % by Weight* |
|---|---|---|
| WATER | 7732-18-5 | 94-89.09 |
| CALCIUM CHLORIDE | 10043-52-4 | 6 |
| SODIUM BENZOATE | 532-32-1 | 0-2 |
| METHYLPARABEN | 99-76-3 | 0-2 |
| Erythrosine | 16423-68-0 | 0-0.01 |

| | | |
|---|---|---|
| (*add up to 100%) | | |

Component 2 is in an embodiment provided in a form indicated above. In use. a few drops of component 2 is added to for instance regular tap water. This solution is subsequently provided for gelling the first component.

In an embodiment, component 1 and component 2 are provided in a kit-of-parts. Component 1 is for instance the aqueous composition provided in various colours in tubes. The component 2 is provided in the illustrated, concentrated form in for instance a small bottle. A measuring cup or bowl can be provided with an indication of the amount of component 2 and the required amount of (regular tap) water. The cup or bowl is dimensioned to properly holed a filled casting mould.

It will also be clear that the above description and drawings are included to illustrate some embodiments of the invention, and not to limit the scope of protection. Starting from this disclosure, many more embodiments will be evident to a skilled person. These embodiments are within the scope of protection and the essence of this invention and are obvious combinations of prior art techniques and the disclosure of this patent.

### Reference numbers

1 casting mould
2 first casting mould sub volume
3 second casting mould sub volume
4 casting mould outer wall
5 first casting mould sub volume floor
6 separating wall
7 second casting mould sub volume floor
8 indented volume
10 gel object
11 main body
12 sub body
13 further sub body
H casting mould outer wall height
S separating wall height
D indent depth

## Claims

1. A method for casting a gel object, comprising providing:
- at least two gel-forming compositions, and
- a casting mould, said casting mould comprising a casting mould outer wall having a casting mould outer wall height and enclosing a casting mould volume, said casting mould volume divided into a first casting mould sub volume that is separated from at least one second casting mould sub volume through a separating wall having a separating wall height that is lower than said casting mould outer wall height,
said method further comprising:
- filling said at least one second casting mould sub volume with a first of said at least two gel-forming compositions;
- filling said first casting mould sub volume with a second of said at least two gel-forming compositions, and
- allowing said gelling compositions to form into a gel providing a gel object comprising a main body of said second of said at least two gel-forming compositions and at least one connected sub body of said first of said at least two gel-forming compositions.

2. The method of claim 1, wherein said at least two gel-forming compositions have different colours, in particular including one colourless gel-forming composition.

3. The method of claim 1 or 2, wherein providing said at least two gel-forming compositions comprising providing:
- at least two first aqueous compositions comprising a water-solvable salt of an alginic acid and at least one of a respective first and second colouring agent or colorant;
- a second aqueous composition comprising at least 0.5-10 % by wt. calcium chloride, and
- contacting said at least two first aqueous compositions and said second aqueous composition.

4. The method of claim 3, further comprising:
- filling said at least one second casting mould sub volume with a first of said first aqueous solution;
- filling said first casting mould sub volume with a second of said first aqueous solution, and
- contacting said first aqueous solutions in said casting mould with said second aqueous solution.

5. A kit-of-parts comprising:
- at least one casting mould comprising a casting mould outer wall having a casting mould outer wall height and enclosing a casting mould volume, said casting mould volume divided into a first casting mould sub volume that is separated from at least one second casting mould sub volume through a separating wall having a separating wall height that is lower than said casting mould outer wall height;
- at least two first aqueous compositions comprising a water-soluble alginate, in particular sodium alginate, in an amount of between 1 and 4 % by wt. and at least one of said at least two first aqueous compositions comprising a colouring agent, said at least two first aqueous compositions provided in a respective first and second container;
- a second aqueous composition comprising a gelling compound, in particular calcium chloride, said second aqueous composition comprising an amount of between 5 and 10 % by wt. calcium chloride and is provided in a further container.

6. The kit-of-parts of claim 5, wherein said at least two first aqueous compositions each comprises at least one colouring agent providing said two first aqueous compositions with a visually different colour.

7. The kit-of-parts of claim 5 or 6, wherein said at least two first aqueous compositions are partially gelled, in particular said at least two first aqueous compositions are each provided in a tube and gelled such that they need to be pressed out of their tube by mild pressure, for instance by hand.

8. The kit-of-parts of any one of claims 5-7, the casting mould comprising a series of second casting mould sub volumes that are each separated from said first casting mould sub volume via a said separating wall.

9. The kit-of-parts of any one of claims 5-8, wherein said casting mould sub volumes each comprise a casting mould sub volume floor, wherein in particular said a casting mould sub volume floor is raised a maximum of 20 % of the outer wall height with respect to a neighbouring sub volume floor.

10. The kit-of-parts of any one of claims 5-9, wherein at least one sub volume comprises an indent or hole, in particular having a depth of between 1-0.25 times the separating wall height.

11. The kit-of-parts of any one of claims 5-10, wherein the casting mould has a ratio of casting mould diameter to casting mould outer wall height of between 1:1 to 20:1, and a ratio of casting mould outer wall height to separating wall height of between 3:1 to 3:2.

12. The kit-of-parts of any one of claims 5-11, wherein the casting mould diameter is between 3 and 15 cm, in particular between 5 and 9 cm.

## Patentansprüche

1. Verfahren zum Gießen eines Gelobjekts, umfassend das Bereitstellen von:
- mindestens zwei gelbildende Zusammensetzungen und
- eine Gussform, wobei die Gussform eine Gussformaußenwand mit einer Gussformaußenwandhöhe aufweist und ein Gussformvolumen umschließt, wobei das Gussformvolumen in ein erstes Gussformuntervolumen unterteilt ist, das von mindestens einer zweiten Gussform getrennt ist Teilvolumen durch eine Trennwand mit einer Trennwandhöhe, die geringer ist als die Außenwandhöhe der Gießform,
wobei das Verfahren weiterhin umfasst:
- Füllen des mindestens einen zweiten Gussform-Untervolumens mit einer ersten der mindestens zwei gelbildenden Zusammensetzungen;
- Füllen des ersten Gussform-Untervolumens mit einer zweiten der mindestens zwei gelbildenden Zusammensetzungen und
- Zulassen, dass sich die gelbildenden Zusammensetzungen zu einem Gel formen, wodurch ein Gelgegenstand bereitgestellt wird, der einen Hauptkörper der zweiten der mindestens zwei gelbildenden Zusammensetzungen und mindestens einen verbundenen Unterkörper der ersten der mindestens zwei gelbildenden Zusammensetzungen umfasst.

2. Verfahren nach Anspruch 1, wobei die mindestens zwei gelbildenden Zusammensetzungen unterschiedliche Farben haben, insbesondere einschließlich einer farblosen gelbildenden Zusammensetzung.

3. Verfahren nach Anspruch 1 oder 2, wobei die mindestens zwei gelbildenden Mittel bereitgestellt werden
Zusammensetzungen, die Folgendes umfassen:
- mindestens zwei erste wässrige Zusammensetzungen, die ein wasserlösliches Salz einer Alginsäure und mindestens einen ersten und zweiten Farbstoff umfassen;
- eine zweite wässrige Zusammensetzung, die mindestens 0,5-10 Gew.-% Calciumchlorid enthält und
- Kontaktieren der mindestens zwei ersten wässrigen Zusammensetzungen und der zweiten wässrigen Zusammensetzung.

4. Verfahren nach Anspruch 3, weiterhin umfassend:
- Füllen des mindestens einen zweiten Gussform-Untervolumens mit einer ersten der ersten wässrigen Lösung;
- Füllen des ersten Gussform-Untervolumens mit einer zweiten der ersten wässrigen Lösung und
- Inkontaktbringen der ersten wässrigen Lösungen in der Gussform mit der zweiten wässrigen Lösung.

5. Ein Kit-of-parts umfassend:
- mindestens eine Gussform, die eine Gussformaußenwand mit einer Gussformaußenwandhöhe aufweist und ein Gussformvolumen umschließt, wobei das Gussformvolumen in ein erstes Gussformuntervolumen unterteilt ist, das von mindestens einem zweiten Gussformuntervolumen durch eine Trennwand getrennt ist Wand mit einer Trennwandhöhe, die niedriger ist als die Außenwandhöhe der Gießform;
- mindestens zwei erste wässrige Zusammensetzungen enthaltend ein wasserlösliches Alginat, insbesondere Natriumalginat, in einer Menge zwischen 1 und 4 Gew.-%. und mindestens eine der mindestens zwei ersten wässrigen Zusammensetzungen umfasst ein Färbemittel, wobei die mindestens zwei ersten wässrigen Zusammensetzungen in einem jeweiligen ersten und zweiten Behälter bereitgestellt werden;
- eine zweite wässrige Zusammensetzung, die eine gelierende Verbindung, insbesondere Calciumchlorid, umfasst, wobei die zweite wässrige Zusammensetzung eine Menge zwischen 5 und 10 Gew.-% umfasst. Calciumchlorid und wird in einem weiteren Behälter bereitgestellt.

6. Kit-of-parts nach Anspruch 5, wobei die mindestens zwei ersten wässrigen Zusammensetzungen jeweils mindestens ein Färbemittel umfassen, das den beiden ersten wässrigen Zusammensetzungen eine optisch unterschiedliche Farbe verleiht.

7. Kit-of-parts nach Ansprüche 5 oder 6, wobei die mindestens zwei ersten wässrigen Zusammensetzungen teilweise geliert sind, insbesondere werden die mindestens zwei ersten wässrigen Zusammensetzungen jeweils in einer Tube bereitgestellt und so geliert, dass sie durch leichten Druck, beispielsweise von Hand, aus ihrer Tube gedrückt werden müssen.

8. Kit-of-parts nach eine der Ansprüche 5-7, umfassend eine Reihe zweiter Gussformuntervolumen, die jeweils über eine Trennwand von dem ersten Gussformuntervolumen getrennt sind.

9. Kit-of-parts nach eine der Ansprüche 5-8, wobei die Gussformuntervolumen jeweils einen Gussformuntervolumenboden umfassen, wobei insbesondere der Gussformuntervolumenboden um maximal 20 % der Außenwandhöhe in Bezug auf a erhöht ist anliegenden Untervolumenboden.

10. Kit-of-parts nach eine der Ansprüche 5-9, wobei mindestens ein Teilvolumen eine Vertiefung oder ein Loch umfasst, insbesondere mit einer Tiefe zwischen dem 1-0,25-fachen der Trennwandhöhe.

11. Kit-of-parts nach eine der Ansprüche 5-10, wobei die Gussform ein Verhältnis von Gussformdurchmesser zu Gussformaußenwandhöhe zwischen 1:1 und 20:1 und ein Verhältnis von Gussformaußenwandhöhe zu Trennwandhöhe von aufweist zwischen 3:1 und 3:2.

12. Kit-of-parts nach eine der Ansprüche 5-11, wobei der Gießformdurchmesser zwischen 3 und 15 cm, insbesondere zwischen 5 und 9 cm, beträgt.

## Revendications

1. Procédé pour couler un objet en gel, comprenant fournir:
- au moins deux compositions gélifiantes, et
- un moule de coulée, ledit moule de coulée comprenant une paroi extérieure de moule de coulée ayant une hauteur de paroi extérieure de moule de coulée et renfermant un volume de moule de coulée, ledit volume de moule de coulée étant divisé en un premier sous-volume de moule de coulée qui est séparé d'au moins un second moule de coulée un sous-volume à travers une paroi de séparation ayant une hauteur de paroi de séparation qui est inférieure à ladite hauteur de paroi extérieure du moule de coulée,
ledit procédé comprenant en outre :
- remplir ledit au moins un second sous-volume de moule de coulée avec une première desdites au moins deux compositions gélifiantes ;
- remplissage dudit premier sous-volume de moule de coulée avec une seconde desdites au moins deux compositions formant un gel, et
- laisser lesdites compositions gélifiantes se former en un gel fournissant un objet en gel comprenant un corps principal de ladite deuxième desdites au moins deux compositions gélifiantes et au moins un sous-corps connecté de ladite première desdites au moins deux compositions gélifiantes.

2. Procédé selon la revendication 1, dans lequel lesdites au moins deux compositions gélifiantes ont des couleurs différentes, en particulier comprenant une composition gélifiante incolore.

3. Procédé selon la revendication 1 ou 2, dans lequel la fourniture desdites au moins deux substances compositions gélifiantes comprenant fournir:
- au moins deux premières compositions aqueuses comprenant un sel soluble dans l'eau d'un acide alginique et au moins l'un d'un premier et second agent colorant ou colorant respectif ;
- une seconde composition aqueuse comprenant au moins 0,5 à 10 % en poids. chlorure de calcium, et
- mettre en contact lesdites au moins deux premières compositions aqueuses et ladite seconde composition aqueuse.

4. Procédé selon la revendication 3, comprenant en outre :
- remplir ledit au moins un second sous-volume de moule de coulée avec une première de ladite première solution aqueuse ;
- remplir dudit premier sous-volume de moule de coulée avec une seconde de ladite première solution aqueuse, et
- mettre en contact lesdites premières solutions aqueuses dans ledit moule de coulée avec ladite seconde solution aqueuse.

5. Un kit de pièces comprenant :
- au moins un moule de coulée comprenant une paroi extérieure de moule de coulée ayant une hauteur de paroi extérieure de moule de coulée et renfermant un volume de moule de coulée, ledit volume de moule de coulée étant divisé en un premier sous-volume de moule de coulée qui est séparé d'au moins un deuxième sous-volume de moule de coulée par une séparation paroi ayant une hauteur de paroi de séparation qui est inférieure à ladite hauteur de paroi externe du moule de coulée;
- au moins deux premières compositions aqueuses comprenant un alginate hydrosoluble, notamment de l'alginate de sodium, en une quantité comprise entre 1 et 4 % en poids. et au moins l'une desdites au moins deux premières compositions aqueuses comprenant un agent colorant, lesdites au moins deux premières compositions aqueuses fournies dans un premier et un second récipient respectifs ;
- une deuxième composition aqueuse comprenant un composé gélifiant, notamment du chlorure de calcium, ladite deuxième composition aqueuse comprenant une quantité comprise entre 5 et 10 % en poids. chlorure de calcium et est fourni dans un autre récipient.

6. Le kit de pièces selon la revendication 5, dans lequel lesdites au moins deux premières compositions aqueuses comprennent chacune au moins un agent colorant conférant auxdites deux premières compositions aqueuses une couleur visuellement différente.

7. Le kit de pièces selon la revendication 5 ou 6, dans lequel lesdites au moins deux premières solutions aqueuses sont partiellement gélifiées, en particulier lesdites au moins deux premières compositions aqueuses sont fournies chacune dans un tube et gélifiées de sorte qu'elles doivent être pressées hors de leur tube par une légère pression, par exemple à la main.

8. Le kit de pièces selon une des revendications 5-7, comprenant une série de deuxièmes sous-volumes de moule de coulée qui sont chacun séparés dudit premier sous-volume de moule de coulée via une dite paroi de séparation.

9. Le kit de pièces selon une des revendications 5-8, dans lequel lesdits sous-volumes de moule de coulée comprennent chacun un plancher de sous-volume de moule de coulée, dans lequel en particulier ledit plancher de sous-volume de moule de coulée est surélevé d'un maximum de 20 % de la hauteur de paroi extérieure par rapport à un plancher de sous-volume voisin.

10. Le kit de pièces selon une des revendication 5-9, dans lequel au moins un sous-volume comprend un renfoncement ou un trou, ayant en particulier une profondeur comprise entre 1 et 0,25 fois la hauteur de la paroi de séparation.

11. Le kit de pièces selon une des revendications 5-10, dans lequel le moule de coulée a un rapport du diamètre du moule de coulée à la hauteur de la paroi extérieure du moule de coulée compris entre 1 : 1 et 20 : 1, et un rapport de la hauteur de la paroi extérieure du moule de coulée à la hauteur de la paroi de séparation de entre 3 : 1 et 3 : 2.

12. Le kit de pièces selon une des revendications 5-11, dans lequel le diamètre du moule de coulée est compris entre 3 et 15 cm, en particulier entre 5 et 9 cm.
